

June 28, 1960

J. W. MAUSTELLER

2,943,034

INHIBITORS TO TRANSFER OF STRUCTURAL MATERIAL  
CONSTITUENTS IN LIQUID SODIUM

Filed Oct. 19, 1955



INVENTOR.  
JOHN W. MAUSTELLER.

BY

*Brown, Atchley, Flick & Leckham*  
*bis*  
ATTORNEYS.

1

2,943,034

## INHIBITORS TO TRANSFER OF STRUCTURAL MATERIAL CONSTITUENTS IN LIQUID SODIUM

John W. Mausteller, Evans City, Pa., assignor to Mine Safety Appliances Company, Pittsburgh, Pa., a corporation of Pennsylvania

Filed Oct. 19, 1955, Ser. No. 541,511

8 Claims. (Cl. 204—154.2)

This invention relates to inhibitors which will decrease the mass transfer of structural material constituents in liquid sodium and in particular it relates to inhibitors which will decrease the mass transfer of those radioactive species having a longer half life than sodium-24, found in structural materials such as stainless steel, mild steel, Inconel and similar alloys used to transport liquid sodium in a nuclear reactor.

Liquid sodium is used as a heat transfer medium in nuclear reactors. The sodium is circulated through stainless steel pipe or other alloy pipe containing various constituents such as manganese, cobalt, iron, antimony and tantalum which may become radioactive. These constituents tend to dissolve in the liquid sodium and are circulated throughout the cooling system of the nuclear reactor. These constituents thereafter deposit on the piping outside the reactor and present a radiation hazard. Thus, the mass transfer of radioactive constituents found in these structural materials can create a serious problem in reactor maintenance. The oxygen content of liquid sodium has been found to have a decided effect on the mass transfer of radioactive constituents found in stainless steel, Inconel and similar alloys. In order to hold the mass transfer of these constituents to a minimum, it is necessary in liquid sodium systems of this type to maintain the oxygen content of the sodium below 0.01 wt. percent and preferably below 0.005 wt. percent. However, the relatively small difference in oxygen concentration of 0.003 and 0.01 wt. percent will produce an increase in transfer of 3 to 54 fold depending upon the isotope transferred. Thus, it has become important to find inhibitors which will decrease or completely prevent the transfer of these radioactive constituents such as cobalt-60, tantalum-182, manganese-54, iron-59 and antimony-124 in liquid sodium.

One object of this invention is to provide materials which will inhibit the transfer of structural material constituents in liquid sodium.

Another object is to provide inhibitors which will decrease or prevent the mass transfer of radioactive constituents having a longer half life than sodium-24 which are found in structural materials used to transport liquid sodium.

Other objects will become apparent from time to time throughout the following specification and appended claims.

These inhibitors will be more fully described hereinafter and the novelty thereof will be particularly pointed out and distinctly claimed.

This invention is based upon the discovery that metals such as barium, strontium, calcium, titanium, antimony and magnesium when used in an amount as little as 1 wt. percent in a liquid sodium heat transfer system using stainless steel or other alloy piping will inhibit the mass transfer of radioactive structural material constituents in liquid sodium. Although the mechanism of inhibition is not completely understood, it is believed to be a function

2

of the reduction of oxygen content, surface plating and "salting out" by the inhibitor. Thus, the inhibited species need not be radioactive to be inhibited.

Since the radioactive constituents of structural materials such as stainless steel, Inconel, mild steel and similar alloys having a half life greater than sodium-24 are of particular interest insofar as the inhibition of their transfer in liquid sodium is concerned, the half lives of the more important isotopes as compared to sodium-24 are presented in the table below:

| Isotope:     | Half life |
|--------------|-----------|
| Sodium-24    | 15 hours  |
| Tantalum-182 | 117 days  |
| Iron-59      | 46 days   |
| Manganese-54 | 310 days  |
| Cobalt-60    | 5.2 years |
| Antimony-124 | 60 days   |

It is readily apparent from this table that the radiation hazard of the isotopes listed can last for several months. It is therefore extremely important to prevent these isotopes from being transported in a liquid sodium system used to transfer heat from a nuclear reactor, especially at temperatures above 1200° F. where mass transfer has been found to increase at an exponential rate.

The attached drawing shows typical apparatus in which the invention may be carried out.

The experimental apparatus for testing the effectiveness of various metals as inhibitors of isotope transfer in a liquid sodium system consisted of a loop constructed of ½" stainless steel pipe which was large enough to contain 450 g. of sodium. The bottom of the loop was equipped with a 12" length of ½" stainless steel pipe opening into the loop at its upper end and closed at its lower end and operable as a cold trap for oxide impurities as described in the copending application of Batutis and Walters, Serial No. 538,447, filed October 4, 1955, now Patent No. 2,879,157, issued March 3, 1959. A drain valve was also inserted in the bottom of the loop adjacent the cold trap. A 1½" stainless steel pipe connected to the top of the loop served as an expansion tank. This tank was fitted with a 1½" gate valve for sampling and access to the radioactive source. Two rod-type heaters were inserted in the top of the loop adjacent the expansion tank to supply heat to the system. One leg of the loop was insulated and the other leg was not. The temperature of the liquid sodium was obtained from a thermocouple located in the bottom of the expansion tank. Circulation of the liquid sodium was maintained by thermal convection.

The operating procedure used to test various metals as transfer inhibitors in the apparatus described was as follows: the loop was cleaned with a 8:1:1 mixture of water, nitric acid and hydrochloric acid, rinsed with water and evacuated to dryness. All valves were disassembled, cleaned with naphtha, dried and reassembled. The loop was then filled with 450 g. of sodium filtered at 350° F. This method of cleaning and filling usually resulted in an original oxygen content of less than 0.005 wt. percent. If the oxygen content was greater than this value, a short period of cold trapping would remedy the situation. The cold, uninsulated leg of the loop was heated with a torch to melt the sodium and 1 wt. percent of inhibitor was added through the gate valve. When the temperature of the liquid sodium reached 1000° ±15° F., the radioactive source was inserted through the gate valve. The entire system was operated at this temperature for 30 days. At the end of this time, the radioactive source was removed through the gate valve into an argon-filled glass apparatus. The liquid sodium was drained from the system at 1000° F., to prevent pre-

cipitation of dissolved materials on the pipe walls. After cooling the loop to room temperature, the cold trap was removed and methanol was added to the loop until all reaction ceased as indicated by hydrogen bubbles. Water was finally flushed through the system to remove residual caustic. Tests of the methanol and water showed that no significant amounts of radioactive material were removed from the walls. Sections of the stainless steel pipe were cut out, flattened, and tested for radioactivity with a radiation counter. The radiation count of each test specimen was compared with the radiation count of a control treated in the same manner except that no inhibitor was added. All inhibitors were rated on the basis of an inhibitor factor calculated as gross radiation count on the control divided by gross radiation count on the sample. Thus, the higher the factor, the better the inhibitor. A factor lower than 1 indicates acceleration of mass transfer.

Several metals were tested and rated as inhibitors with the following results:

| Inhibitor | Inhibitor Factor | Loop Surface           |
|-----------|------------------|------------------------|
| Barium    | 17               | slight dark coating.   |
| Strontium | 12               | no visible coating.    |
| Calcium   | 10               | no visible coating.    |
| Titanium  | 6.4              | heavy silvery coating. |
| Antimony  | 5.7              | dark coating.          |
| Magnesium | 5.6              | slight dark coating.   |
| Tin       | 2.7              | no visible coating.    |
| Bismuth   | 0.87             | no visible coating.    |
| Beryllium | 0.67             | no visible coating.    |
| Germanium | 0.36             | dense silvery coating. |
| Copper    | 0.22             | heavy black coating.   |
| Zinc      | 0.13             | very slight coating.   |

From the results obtained, it is obvious that barium was the best inhibitor of all the metals tested followed by strontium, calcium, titanium, antimony and magnesium in that order. All the elements in Group IIA of the periodic table were good inhibitors except beryllium. 40 The most significant feature of the good inhibitors was that they were predominantly those which would reduce sodium oxide and apparently formed a protective film on loop surfaces.

Although 1 wt. percent of inhibitors was used in the experiments described, it should be understood that other concentrations may be used if desired. Analyses of materials transported in several of the tests showed that the inhibition of specific isotopes is dependent upon the inhibitor used. Thus, a combination of two or more 45

of the inhibitors disclosed is also considered to be within the spirit and scope of the present invention.

Having thus described this invention fully and completely as required by the patent laws, what is desired 5 to be claimed and secured by United States patent is:

1. The combination with a heat exchange system adjacent a radio-active source wherein liquid sodium is used as a heat transfer medium to absorb heat near said radio-active source, and from which heat is extracted at a point more remote from said source, of a small amount 10 of a metal dissolved in said liquid sodium, said metal being selected from the group, consisting of barium, strontium, calcium, titanium, antimony and magnesium.
2. A combination according to claim 1 in which the metal used is present in about 1 wt. percent of the sodium used.
- 15 3. A combination according to claim 2 in which the metal used is barium.
4. A combination according to claim 2 in which the metal used is strontium.
- 20 5. A combination according to claim 2 in which the metal used is calcium.
6. A combination according to claim 2 in which the metal used is titanium.
- 25 7. A combination according to claim 2 in which the metal used is magnesium.
8. A method of inhibiting mass transfer of radioactive elements, which have a half-life longer than that of sodium-24, in a circulating stream of molten sodium where- 30 in said molten sodium is first heated and then cooled during circulation, which comprises incorporating in said molten sodium a small amount of a metal, said amount being effective to inhibit mass transfer in said sodium, selected from the group consisting of barium, strontium, calcium, titanium, antimony and magnesium.
- 35

#### References Cited in the file of this patent

#### UNITED STATES PATENTS

1,837,744 Zworykin \_\_\_\_\_ Dec. 22, 1931

#### FOREIGN PATENTS

648,293 Great Britain \_\_\_\_\_ Jan. 3, 1951

#### OTHER REFERENCES

Smithells: "Metals Reference Book," Interscience Publishers, Inc. (1949), page 335.

"Liquid Metals Handbook, Sodium (NaK) Supplement," sponsored by Atomic Energy Commission and the Bureau of Ships, Dept. of the Navy, 3rd edition, June 50 1955, pages 13-18, 146.